



US005387496A

**United States Patent** [19]

DeBoer

[11] **Patent Number:** **5,387,496**[45] **Date of Patent:** **Feb. 7, 1995**[54] **INTERLAYER FOR LASER ABLATIVE IMAGING**[75] Inventor: **Charles D. DeBoer, Rochester, N.Y.**[73] Assignee: **Eastman Kodak Company, Rochester, N.Y.**[21] Appl. No.: **99,972**[22] Filed: **Jul. 30, 1993**[51] Int. Cl.<sup>6</sup> ..... **G03C 5/16; G03C 7/26**[52] U.S. Cl. ..... **430/322; 430/201; 430/271; 430/334; 430/944; 430/945; 430/464; 346/76 L; 503/227; 347/264**[58] **Field of Search** ..... **430/201, 270, 271, 944, 430/945, 964, 269, 334, 332; 503/227; 346/76 L**[56] **References Cited****U.S. PATENT DOCUMENTS**

4,973,572 11/1990 DeBoer ..... 503/227

5,171,650 12/1992 Ellis et al. ..... 430/20

*Primary Examiner*—Richard L. Schilling*Attorney, Agent, or Firm*—Harold E. Cole[57] **ABSTRACT**

A process of forming a single color, dye ablation image having an improved D-min comprising imagewise heating by means of a laser, a dye-ablative recording element comprising a support having thereon a dye layer comprising an image dye dispersed in a polymeric binder and an infrared-absorbing material, the laser exposure taking place through the dye side of the element, and removing the ablated image dye material to obtain an image in the dye-ablative recording element, and wherein the element contains an interlayer containing infrared-absorbing material and which is located between the support and the dye layer.

**7 Claims, No Drawings**

## INTERLAYER FOR LASER ABLATIVE IMAGING

This invention relates to the use of an interlayer in a laser dye-ablative recording element.

In recent years, thermal transfer systems have been developed to obtain prints from pictures which have been generated electronically from a color video camera. According to one way of obtaining such prints, an electronic picture is first subjected to color separation by color filters. The respective color-separated images are then converted into electrical signals. These signals are then operated on to produce cyan, magenta and yellow electrical signals. These signals are then transmitted to a thermal printer. To obtain the print, a cyan, magenta or yellow dye-donor element is placed face-to-face with a dye-receiving element. The two are then inserted between a thermal printing head and a platen roller. A line-type thermal printing head is used to apply heat from the back of the dye-donor sheet. The thermal printing head has many heating elements and is heated up sequentially in response to the cyan, magenta and yellow signals. The process is then repeated for the other two colors. A color hard copy is thus obtained which corresponds to the original picture viewed on a screen. Further details of this process and an apparatus for carrying it out are contained in U.S. Pat. No. 4,621,271, the disclosure of which is hereby incorporated by reference.

Another way to thermally obtain a print using the electronic signals described above is to use a laser instead of a thermal printing head. In such a system, the donor sheet includes a material which strongly absorbs at the wavelength of the laser. When the donor is irradiated, this absorbing material converts light energy to thermal energy and transfers the heat to the dye in the immediate vicinity, thereby heating the dye to its vaporization temperature for transfer to the receiver. The absorbing material may be present in a layer beneath the dye and/or it may be admixed with the dye. The laser beam is modulated by electronic signals which are representative of the shape and color of the original image, so that each dye is heated to cause volatilization only in those areas in which its presence is required on the receiver to reconstruct the color of the original object. Further details of this process are found in GB 2,083,726A, the disclosure of which is hereby incorporated by reference.

In one ablative mode of imaging by the action of a laser beam, an element with a dye layer composition comprising an image dye, an infrared-absorbing material, and a binder coated onto a substrate is imaged from the dye side. The energy provided by the laser drives off the image dye at the spot where the laser beam hits the element and leaves the binder behind. In ablative imaging, the laser radiation causes rapid local changes in the imaging layer thereby causing the material to be ejected from the layer. This is distinguishable from other material transfer techniques in that some sort of chemical change (e.g., bond-breaking), rather than a completely physical change (e.g., melting, evaporation or sublimation), causes an almost complete transfer of the image dye rather than a partial transfer. The transmission D-min density value serves as a measure of the completeness of image dye removal by the laser.

U.S. Pat. No. 4,973,572 relates to infrared-absorbing cyanine dyes used in laser-induced thermal dye transfer elements. In Example 3 of that patent, a positive image

is obtained in the dye element by using an air stream to remove sublimed dye. However, there is no disclosure of the use of an interlayer containing infrared-absorbing material in the element in this process.

5 U.S. Pat. No. 5,171,650 relates to an ablation-transfer image recording process. In that process, an element is employed which contains a dynamic release layer which absorbs imaging radiation which in turn is over-coated with an ablative carrier topcoat. An image is 10 transferred to a receiver in contiguous registration therewith. The useful image obtained in this process is contained on the receiver element. However, there is no disclosure in that patent that a useful positive image can be obtained in the recording element or of a single-sheet 15 process.

It is an object of this invention to provide a process for improving the D-min obtained in a dye-ablative recording element. It is another object of this invention to provide a single-sheet process which does not require 20 a separate receiving element.

These and other objects are achieved in accordance with the invention which comprises a process of forming a single color, dye ablation image having an improved D-min comprising imagewise heating by means of a laser, a dye-ablative recording element comprising a support having thereon a dye layer comprising an image dye dispersed in a polymeric binder and an infrared-absorbing material, the laser exposure taking place through the dye side of the element, and removing the ablated image dye material to obtain an image in the dye-ablative recording element, and wherein the element contains an interlayer containing infrared-absorbing material and which is located between the support and the dye layer.

30 35 It has been found unexpectedly that use of an interlayer containing infrared-absorbing material in the above dye-ablative recording element for laser ablative imaging significantly affects the desired dye cleanout as evidenced by the resulting faster writing speeds to achieve a given minimum density. Minimum densities of 40 less than 0.10 are achieved in accordance with the invention.

The interlayer of the dye-ablative recording element 45 employed in the process of this invention can be coated with or without a binder. If a binder is employed, it is preferably a hydrophilic material such as, for example, gelatin, poly(vinyl alcohol), hydroxyethyl cellulose, poly(vinyl pyrrolidone), casein, albumin, guar gum, and the like. In a preferred embodiment of the invention, the hydrophilic binder is poly(vinyl alcohol) or nitrocellulose. When the hydrophilic binder is present, good results have been obtained at a concentration of from about 0.01 to about 1.0 g/m<sup>2</sup>.

50 55 The dye ablation process of this invention can be used to obtain medical images, reprographic masks, printing masks, etc. The image obtained can be a positive or a negative image.

Any polymeric material may be used as the binder in the recording element employed in the process of the 60 invention. For example, there may be used cellulosic derivatives, e.g., cellulose nitrate, cellulose acetate hydrogen phthalate, cellulose acetate, cellulose acetate propionate, cellulose acetate butyrate, cellulose triacetate, a hydroxypropyl cellulose ether, an ethyl cellulose ether, etc., polycarbonates; polyurethanes; polyesters; poly(vinyl acetate); polystyrene; poly(styrene-co-acrylonitrile); a polysulfone; a poly(phenylene oxide); a poly(ethylene oxide); a poly(vinyl alcohol-co-acetal)

such as poly (vinyl acetal), poly (vinyl alcohol-co-butyl) or poly(vinyl benzal); or mixtures or copolymers thereof. The binder may be used at a coverage of from about 0.1 to about 5 g/m<sup>2</sup>.

In a preferred embodiment, the polymeric binder used in the recording element employed in the process of the invention has a polystyrene equivalent molecular weight of at least 100,000 as measured by size exclusion chromatography, as described in copending U.S. application Ser. No. 08/099,968 filed Jul. 30, 1993 by Kaszczuk and Topel and entitled, "HIGH MOLECULAR WEIGHT BINDERS FOR LASER ABLATIVE IMAGING".

In another preferred embodiment, the infrared-absorbing material employed in the recording element used in the invention is a dye which is employed in the image dye layer/and or in the interlayer. In still another preferred embodiment, the infrared-absorbing material is employed at a concentration of greater than about 0.1 g/m<sup>2</sup> whether in the dye layer or in the interlayer.

To obtain a laser-induced, dye-ablative image using the process of the invention, a diode laser is preferably employed since it offers substantial advantages in terms of its small size, low cost, stability, reliability, ruggedness, and ease of modulation. In practice, before any laser can be used to heat a dye-ablative recording element, the element must contain an infrared-absorbing material, such as cyanine infrared-absorbing dyes as described in U.S. Pat. No. 4,973,572, or other materials as described in the following U.S. Pat. Nos. 4,948,777, 30 4,950,640, 4,950,639, 4,948,776, 4,948,778, 4,942,141, 4,952,552, 5,036,040, and 4,912,083, the disclosures of which are hereby incorporated by reference. As noted above, the infrared-absorbing material is contained in either the image dye layer, the interlayer, or both. The 35 laser radiation is then absorbed into the dye layer and converted to heat by a molecular process known as internal conversion. Thus, the construction of a useful dye layer will depend not only on the hue, transferability and intensity of the image dyes, but also on the ability of the dye layer to absorb the radiation and convert it to heat. As noted above, the laser exposure in the process of the invention takes place through the dye side of the dye ablative recording element, which enables this process to be a single-sheet process, i.e., a separate receiving element is not required.

Lasers which can be used in the invention are available commercially. There can be employed, for example, Laser Model SDL-2420-H2 from Spectra Diode Labs, or Laser Model SLD 304 V/W from Sony Corp.

Any dye can be used in the dye-ablative recording element employed in the invention provided it can be ablated by the action of the laser. Especially good results have been obtained with dyes such as anthraquinone dyes, e.g., Sumikaron Violet RS® (product of 55 Sumitomo Chemical Co., Ltd.), Dianix Fast Violet 3RFS® (product of Mitsubishi Chemical Industries, Ltd.), and Kayalon Polyol Brilliant Blue N-BGM® and KST Black 146® (products of Nippon Kayaku Co., Ltd.); azo dyes such as Kayalon Polyol Brilliant Blue BM®, Kayalon Polyol Dark Blue 2BM®, and KST Black KR® (products of Nippon Kayaku Co., Ltd.), Sumikaron Diazo Black 5G® (product of 60 Sumitomo Chemical Co., Ltd.), and Miktazel Black 5GH® (product of Mitsui Toatsu Chemicals, Inc.); direct dyes such as Direct Dark Green B® (product of Mitsubishi Chemical Industries, Ltd.) and Direct Brown M® and Direct Fast Black D® (products of

Nippon Kayaku Co. Ltd.); acid dyes such as Kayanol Milling Cyanine 5R® (product of Nippon Kayaku Co. Ltd.); basic dyes such as Sumiacryl Blue 6G® (product of Sumitomo Chemical Co., Ltd.), and Aizen Malachite Green® (product of Hodogaya Chemical Co., Ltd.);



or any of the dyes disclosed in U.S. Pat. Nos. 4,541,830, 4,698,651, 4,695,287, 4,701,439, 4,757,046, 4,743,582, 4,769,360, and 4,753,922, the disclosures of which are hereby incorporated by reference. The above dyes may be employed singly or in combination. The dyes may be used at a coverage of from about 0.05 to about 1 g/m<sup>2</sup> and are preferably hydrophobic.

The dye layer of the dye-ablative recording element employed in the invention may be coated on the support or printed thereon by a printing technique such as a gravure process.

Any material can be used as the support for the dye-ablative recording element employed in the invention provided it is dimensionally stable and can withstand the heat of the laser. Such materials include polyesters such as poly(ethylene naphthalate); poly(ethylene tere-

phthalate); polyamides; polycarbonates; cellulose esters such as cellulose acetate; fluorine polymers such as poly(vinylidene fluoride) or poly(tetrafluoroethylene-cohexafluoropropylene); polyethers such as polyoxy-methylene; polyacetals; polyolefins such as polystyrene, polyethylene, polypropylene or methylpentene polymers; and polyimides such as polyimide-amides and polyether-imides. The support generally has a thickness of from about 5 to about 200  $\mu\text{m}$ . In a preferred embodiment, the support is transparent.

The following examples are provided to illustrate the invention.

#### EXAMPLE 1

To evaluate the effect on D-min of an interlayer containing an IR dye, samples were coated with the same dye combination containing an interlayer with and without an IR dye.

Element 1) A monicolor dye ablative recording element according to the invention was prepared by coating on a 100  $\mu\text{m}$  thick poly(ethylene terephthalate) support the following layers:

- a subbing layer of poly(acrylonitrile-covinylene chloride-co-acrylic acid) (14:79:7 wt. ratio) (0.07 g/m<sup>2</sup>);
- an interlayer of poly(vinyl alcohol) Airvol 30 203 ®, (Air Products and Chemicals Inc.) coated at 0.22 g/m<sup>2</sup>, triethanolamine (0.04 g/m<sup>2</sup>) and IR-1 below (0.07 g/m<sup>2</sup>) from water; and
- a neutral dye formulation containing 0.86 g/m<sup>2</sup> of 1000 sec. viscosity nitrocellulose (Hercules Inc.), 0.13 g/m<sup>2</sup> IR-2 below, 0.26 g/m<sup>2</sup> each of Cyan Dye D-1 and D-2 below, 0.07 g/m<sup>2</sup> each of Yellow Dye D-4 and D-5 below, and 0.09 g/m<sup>2</sup> each of Magenta Dye D-6 and D-7 below, from a 30:70 mixture of n-propanol and methyl isobutyl ketone.

Element 2) A control element was prepared similar to Element 1 except that the interlayer did not have any IR-1.

Element 3) This element was similar to Element 1 except that layer c) contained only Cyan Dye 2 at 0.62 g/m<sup>2</sup>, Yellow Dye 4 at 0.15 g/m<sup>2</sup>, and Magenta Dye 7 at 0.26 g/m<sup>2</sup> instead of the dye mixtures, and IR-2 was present at 0.17 g/m<sup>2</sup>.

Element 4) A control element was prepared similar to Element 3 except that the interlayer did not have any IR-1.

Element 5) This element was similar to Element 1 except that layer c) contained 0.43 g/m<sup>2</sup> of 1000 sec. viscosity nitrocellulose (Hercules Inc.), 0.20 g/m<sup>2</sup> IR-2 below, 0.33 g/m<sup>2</sup> of Cyan Dye D-3 below, 0.85 g/m<sup>2</sup> of Cibaset Brown 2R ® (Ciba-Geigy AG), and 0.86 g/m<sup>2</sup> of Magenta Dye D-7 below, from a 16:16:68 mixture of n-butyl acetate, n-butanol and methyl isoamyl ketone.

Element 6) A control element was prepared similar to Element 5 except that the interlayer did not have any IR-1.

5

6



Cyan Dye D-1



Cyan Dye D-2

15

20

25



Cyan Dye D-3



Yellow Dye D-4



Yellow Dye D-5



Magenta Dye D-6

50

55



Magenta Dye D-7



Liquid UV Dye

65



The above elements were exposed in a laser thermal printer of the type disclosed in U.S. Pat. No. 5,268,708.

The diode lasers employed were Spectra Diode Labs No. SDL-2430, having an integral, attached optical fiber for the output of the laser beam with a wavelength range 800-830 nm and a nominal power output of 250 milliwatts at the end of the optical fiber. The cleaved face of the optical fiber (50  $\mu\text{m}$  core diameter) was imaged onto the plane of the dye-ablative element with a 0.33 magnification lens assembly mounted on a translation stage giving a nominal spot size of 16  $\mu\text{m}$ .

The drum, 53 cm in circumference, was rotated at varying speeds and the imaging electronics were activated to provide exposures at 827  $\text{mJ}/\text{cm}^2$ . The translation stage was incrementally advanced across the dye-ablative element by means of a lead screw turned by a microstepping motor, to give a center-to-center line distance of 10  $\mu\text{m}$  (945 lines per centimeter, or 2400 lines per inch). An air stream was blown over the donor surface to remove the sublimed dye. The measured average total power at the focal plane was 100 mW. The Status A density of the dye layer before imaging was approximately 3.0 and was compared to the residual density after writing a D-min patch at 200 rev./min.

The D-min values for the test pieces were then determined in an X-Rite densitometer Model 310 (X-Rite Co.) and recorded in Table 1 as follows.

TABLE 1

| Element     | IR-1 in Interlayer ( $\text{g}/\text{m}^2$ ) | D-min |
|-------------|----------------------------------------------|-------|
| 1           | yes                                          | 0.02  |
| 2 (control) | none                                         | 0.07  |
| 3           | yes                                          | 0.03  |
| 4 (control) | none                                         | 0.06  |
| 5           | yes                                          | 0.03  |
| 6 (control) | none                                         | 0.05  |

The above results show that the D-min values are consistently lower for all samples containing the water-soluble IR-1 dye in their interlayer, regardless of the number of image dyes present in the image dye layers of the samples tested.

#### EXAMPLE 2

This set of experiments was run to determine the effect of the levels of infrared-absorbing dyes in both imaging dye layer and interlayer as well as the effect on the presence of poly(vinyl alcohol) in the interlayer.

Twelve samples were coated as in Element 1 of Example 1, except that layer c) contained 0.71  $\text{g}/\text{m}^2$  Cyan dye D-3, 1.72  $\text{g}/\text{m}^2$  Cibaset Brown 2R (Ciba-Geigy AG), 0.25  $\text{g}/\text{m}^2$  liquid UV dye shown above, 0.59  $\text{g}/\text{m}^2$  of 1139 sec. viscosity nitrocellulose (Hercules Inc.), and varying amounts of IR-2 as shown in Table 2 below, coated from a 4:1:1 mixture of methyl isoamyl ketone with butyl acetate and butanol; and layer b) contained 0.32  $\text{g}/\text{m}^2$  poly(vinyl alcohol) Elvanol 52-22 (DuPont Corp.), 0.03  $\text{g}/\text{m}^2$  triethanolamine, 0.003  $\text{g}/\text{m}^2$  nonylphenoxy polyglycidol, and varying amounts of IR-1 as shown below in Table 2 coated from water.

These coatings were exposed on an apparatus, similar to the one described in U.S. Ser. No. 799,471, at 15 Hz and 8 mm exposure. The Status A densities of the cleared out area were measured (D-min) using the X-Rite densitometer.

TABLE 2

| ELEMENT | IR-2 IN IMAGE DYE LAYER c) ( $\text{g}/\text{m}^2$ ) | IR-1 IN INTERLAYER b) ( $\text{g}/\text{m}^2$ ) | STATUS A D-MIN |
|---------|------------------------------------------------------|-------------------------------------------------|----------------|
| 7       | 0.25                                                 | 0.22                                            | 0.68           |
| 8       | 0.13                                                 | 0.22                                            | 0.50           |
| 9       | None                                                 | 0.22                                            | 1.13           |
| 10      | 0.08                                                 | 0.16                                            | 0.54           |
| 11      | 0.03                                                 | 0.16                                            | 1.57           |
| 12      | 0.25                                                 | 0.11                                            | 0.35           |
| 13      | 0.13                                                 | 0.11                                            | 0.35           |
| 14      | None                                                 | 0.11                                            | 1.12           |
| 15      | 0.08                                                 | 0.05                                            | 0.44           |
| 16*     | 0.03                                                 | 0.05                                            | 1.49           |
| 17      | 0.24                                                 | None                                            | 0.45           |
| 18      | 0.13                                                 | None                                            | 0.45           |

\*Element 16 was the same as element 15, except that the liquid UV dye concentration in the image dye layer was cut in half.

The Status A Densities show that the best dye clean-out is obtained with a concentration of about 0.11  $\text{g}/\text{m}^2$  of water-soluble infrared-absorbing dye IR-1 in the interlayer, and more than 0.11  $\text{g}/\text{m}^2$  of solvent-coatable, infrared-absorbing dye IR-2 in the image dye layer.

#### EXAMPLE 3

This example was run to establish that no binder is needed for the water-soluble, infrared-absorbing dye in the interlayer.

Element 19) A monocolored dye ablative recording element according to the invention was prepared by coating on a 100  $\mu\text{m}$  thick poly(ethylene terephthalate) support the following layers:

- a) a subbing layer of poly(methylacrylate-co-vinylidene chloride-co-itaconic acid (0.11  $\text{g}/\text{m}^2$ );
- b) an interlayer of Type IV deionized gelatin (1.4  $\text{g}/\text{m}^2$ ) and nonylphenoxy polyglycidol (0.03  $\text{g}/\text{m}^2$ ); and
- c) Cyan dye D-3 (0.29  $\text{g}/\text{m}^2$ ), 0.83  $\text{g}/\text{m}^2$  Cibaset Brown 2R (Ciba-Geigy AG), Magenta Dye D-7 (0.12  $\text{g}/\text{m}^2$ ) IR-2 (0.17  $\text{g}/\text{m}^2$ ) and 1000 sec. viscosity nitrocellulose (Hercules Inc.) (0.42

g/m<sup>2</sup>) coated from a 12.5:12.5:75 n-butanol/isopropyl acetate/methyl isobutyl ketone mixture.

Element 20 was prepared similar to Element 19 except that the interlayer b) was 1.12 g/m<sup>2</sup> of IR-1.

These coatings were exposed on a laser thermal printer as described in U.S. Pat. No. 5,268,708, operating at different revolution speeds. The results of the D-min measurements are shown in Table 3.

TABLE 3

|                                                    | 150<br>RPM | 200<br>RPM | 250<br>RPM | 300<br>RPM | 400<br>RPM |
|----------------------------------------------------|------------|------------|------------|------------|------------|
| ELEMENT 19<br>(no IR dye in<br>interlayer)         | 0.13       | 0.19       | 0.27       | 0.43       | 1.03       |
| ELEMENT 20<br>(IR in interlayer<br>without binder) | 0.10       | 0.09       | 0.10       | 0.11       | 0.30       |

The above results show that the additional infrared-absorbing dye in a layer below the image dye layer is effective in contributing to improved dye cleanout as measured by the D-min value. The data also show that this improvement is obtained when the hydrophilic poly(vinyl alcohol) binder is omitted.

The invention has been described in detail with particular reference to preferred embodiments thereof, but it will be understood that variations and modifications can be effected within the spirit and scope of the invention.

What is claimed is:

1. A process of forming a single color, dye ablation image having an improved D-min comprising image-wise-heating by means of a laser, a dye-ablative recording element comprising a support having thereon a dye layer comprising an image dye dispersed in a polymeric binder and an infrared-absorbing material, said laser exposure taking place through the dye side of said element, and removing the ablated image dye material to obtain said image in said dye-ablative recording element, wherein said element also contains an interlayer containing poly(vinyl alcohol) and an infrared-absorbing material and which is located between said support and said dye layer.
- 5 10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 9999

1. A process of forming a single color, dye ablation image having an improved D-min comprising image-wise-heating by means of a laser, a dye-ablative recording element comprising a support having thereon a dye layer comprising an image dye dispersed in a polymeric binder and an infrared-absorbing material, said laser exposure taking place through the dye side of said element, and removing the ablated image dye material to obtain said image in said dye-ablative recording element, wherein said element also contains an interlayer containing poly(vinyl alcohol) and an infrared-absorbing material and which is located between said support and said dye layer.
- 5 10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 36